

# United States Patent

[11] 3,616,302

[72] Inventors Kazuya Osawa  
Yokohama;  
Keiichi Shimizu, Tanashi; Takashi  
Takasue, Tokyo, all of Japan

[21] Appl. No. 707,408

[22] Filed Feb. 23, 1968

[45] Patented Oct. 26, 1971

[73] Assignee The Furukawa Electric Company Limited  
Tokyo, Japan

[32] Priorities Feb. 27, 1967

[33] Japan

[31] 42/12427  
Nov. 6, 1967, Japan, No. 42/71334

[54] **INSOLUBLE ANODE FOR ELECTROLYSIS AND A  
METHOD FOR ITS PRODUCTION**  
4 Claims, No Drawings

[52] U.S. Cl..... 204/40,  
204/290 F

[51] Int. Cl..... C23b 5/46

[50] Field of Search..... 204/290,  
290 F, 96, 105.1, 48, 40, 56

[56] **References Cited**  
UNITED STATES PATENTS  
2,631,115 3/1953 Fox .....

Primary Examiner—Howard S. Williams  
Assistant Examiner—Sidney S. Kanter  
Attorney—Stevens, Davis, Miller & Mosher

**ABSTRACT:** An insoluble anode suitable for use in electrolysis and a method for its production are provided. The anode comprises three components which are:

- a. a base substrate treated by sandblasting, said substrate being selected from the group consisting of titanium, zirconium and tantalum or alloys thereof;
- b. a thin metal layer formed on said substrate, said thin metal layer being selected from the group consisting of platinum, palladium and rhodium or alloys thereof; and
- c. an outermost layer of manganese dioxide electroplated on said thin metal layer in an aqueous solution of manganese sulfate containing about 10 to about 30 grams/liter of free sulfuric acid at a current density of about 0.015 to about 0.007 A./dm.<sup>2</sup>.

The anode is produced by sandblasting a base substrate metal of titanium or its alloy to form minute indentations on the surface, electroplating on said base substrate metal a thin layer of platinum, and electrodepositing a layer of manganese dioxide on said thin layer in an aqueous solution of manganese sulfate containing 10–30 g./l. of free sulfuric acid at a current density of 0.015–0.007 A./dm.<sup>2</sup>.

**INSOLUBLE ANODE FOR ELECTROLYSIS AND A  
METHOD FOR ITS PRODUCTION**

The present invention relates to an insoluble anode for use in various kinds of electrolysis.

The principal object of the invention is to provide an insoluble anode having such characteristics that it is less soluble in an electrolyte thus preventing the electrolyte from pollution and is not deposited on a cathode even when it is dissolved in the electrolyte, that it has a low oxygen overvoltage during the electrolysis thus economizing the electric power necessary for the electrolysis, and that it has excellent anode characteristics for electrolytic winning of zinc.

In the electrolytic industry it is the most important problem to select a suitable insoluble anode having such improved characteristics that it does not pollute an electrolyte, and that it has a long life and a low oxygen overvoltage during the electrolysis. It is known that platinum is an excellent anode material which satisfies the above-mentioned characteristics. However, platinum is expensive and hence is not suitable for industrial use, and thus carbon and lead alloy electrodes have generally been used. The carbon anode, however, has the disadvantage that it greatly pollutes the electrolyte, wears fast, and has a high electric resistance which results in an increase in cell voltage. The disadvantage of the lead alloy anode consists in that lead dissolves into the electrolyte and the solute is deposited on the cathode to decrease the purity of the deposit obtained, that the oxygen overvoltage becomes high, and that in case of electrolytic winning of zinc the zinc obtained contains a considerable amount of lead as an impurity. The zinc obtained is less expensive, but it cannot be used as a diecasting material which requires pure zinc.

Under the above circumstances, it has recently been proposed to electroplate the surface of a titanium substrate with platinum and electrodeposit on the electroplated surface with lead dioxide to manufacture an insoluble anode. This anode improved the characteristics somewhat, but has the disadvantage that it has a comparatively high oxygen overvoltage, that lead dioxide is dissolved into certain electrolyte, to soil it, that lead reduced in the electrolyte is deposited together with electrolytic products on the cathode, and that in case of electrolytic winning of zinc, the zinc obtained contains lead as an impurity in the same manner as the aforementioned lead alloy anode.

The invention is based on the recognition that electrodeposited manganese dioxide is an insoluble and electrically conductive oxide which, even when dissolved into an electrolyte, cannot easily be deposited as a reduced product on the cathode. Experiments have yielded such an insoluble anode for use in electrolysis that it is less soluble into an electrolyte and hence does not pollute it, that it is not deposited on a cathode even when dissolved into the electrolyte, that it has a low oxygen overvoltage during the electrolysis to economize the electric power necessary for electrolysis, and that it has an optimum effect when applied to electrolytic winning of zinc.

The invention provides the above-mentioned insoluble anode for use in electrolysis which comprises a base substrate metal of titanium, zirconium, tantalum or an alloy mainly composed thereof sandblasted on the surface, a thin layer of platinum palladium, rhodium, or an alloy mainly composed thereof formed on said substrate metal, and an outermost layer of manganese dioxide electrodeposited on said thin layer.

The electrodeposited manganese dioxide is an insoluble and electrically conductive oxide, while manganese cannot easily be deposited from an aqueous solution and hence gives no disturbance to electrolytic production of zinc. Thus, if use is made of manganese dioxide to produce an insoluble anode for use in electrolysis, it is quite possible to prevent impurities from becoming mixed into an electrolytic product.

The electrodeposited manganese dioxide, however, is very brittle so that it is difficult to form the anode from manganese dioxide itself. Moreover, the electrodeposited manganese dioxide has a large internal stress and is thus liable to be detached from the substrate when it is electrodeposited

thereon to form an anode. Any conventional manganese dioxide electrodeposited on the base substrate metal not only dissolves considerable in an electrolyte, but also causes formation of a passive oxide film on the interface between itself and the substrate metal, and therefore cannot be used for an anode.

The invention provides the possibility of applying the electrodeposited manganese dioxide to an anode without causing the above-mentioned unfavorable properties as a result of various investigations. That is, the invention makes use of a base substrate metal of titanium, zirconium, tantalum, or an alloy mainly composed thereof, sandblasted on the surface. In this case, any metal may be alloyed with titanium, zirconium, or tantalum insofar as it does not adversely affect their corrosion resistance. For example, the alloy of titanium, zirconium, and tantalum or one composed of any of these three metals plus a few percent of palladium or aluminum may be used. This base substrate metal of the invention is capable of decreasing the internal stress of deposits formed on it and electrodepositing the manganese dioxide without causing the above-mentioned unfavorable properties.

The insoluble anode of the invention further comprises a thin layer of platinum, palladium, rhodium, or an alloy mainly composed thereof, formed on the aforementioned base substrate metal. In this case, any metal may be alloyed with platinum, palladium, or rhodium to make the thin layer insofar as it is free from oxidation, for example, the alloy of these three metals. The assembly thus formed renders it possible to prevent formation of a passive oxide film on the interface between the base substrate metal and the electrodeposited manganese dioxide layer formed on the thin alloy layer.

The thickness of the thin layer must be so determined that the minute indentations produced by the sandblast will remain discernible. It is preferable to determine the thickness of the thin alloy layer as 0.01-0.3  $\mu$ .

The invention preferably makes use of titanium or its alloy as the alloy substrate material when the anode of the invention is used for the electrolytic winning of zinc. It is preferable to form a thin layer of platinum or its alloy having a thickness of 0.01-0.3  $\mu$  on the interface between the base substrate metal and the electrodeposited manganese dioxide layer. The reason is that the thickness of less than 0.01  $\mu$  is less effective in preventing the formation of the passive oxide film while the thickness of more than 0.3  $\mu$  not only prevents uniform electrodeposition of manganese dioxide but also makes undiscernible the indentations produced on the surface of the base substrate metal by the sandblast treatment.

As above mentioned the conventional electrodeposited manganese dioxide when used as an anode is liable to be detached from the substrate owing to the internal stress, and dissolved as permanganate ion into the electrolyte. In order to obviate such disadvantages the invention makes use of an aqueous solution of manganese sulfate containing 10-30 g./l. of free sulfuric acid as the composition of the electrolyte to be used in electrodepositing manganese dioxide and of current density of 0.015-0.007 A./dm.<sup>2</sup>.

The above-mentioned conditions for the electrodeposition renders it possible to obtain electrodeposited manganese dioxide which is very hard and dense and has less internal stress, thus improving the adherent property thereof. Moreover, the electrodeposited manganese dioxide has a small electric resistance which permits of decreasing the cell voltage during electrolysis. Moreover, the electrodeposited manganese dioxide is not dissolved into the electrolyte.

If the concentration of the free sulfuric acid lies outside of the above-mentioned range of 10-30 g./l., the electrolytic voltage is gradually increased. When the concentration reaches more than 30 g./l., the electrodeposited manganese dioxide becomes detached from the substrate material. Moreover, when the current density becomes more than 0.05 A./dm.<sup>2</sup>, the cell voltage becomes high and the electrodeposited manganese dioxide is changed into permanganate ion which is soluble in the electrolyte. If the current

density becomes too small, the electrodeposition of manganese dioxide requires a plenty of times so that it is preferable to use the current density of more than 0.005 A./dm.<sup>2</sup>.

It is desirable to make the thickness of the electrodeposited manganese dioxide layer about 10-100  $\mu$ . If the thickness is larger than 100  $\mu$ , the internal stress so increases as to cause the electrodeposited manganese dioxide to be detached from the substrate material, while if the thickness is smaller than 10  $\mu$ , oxygen evolves on the surface of the thin layer which contains a basic composition selected from a group consisting of platinum, palladium and rhodium, and forms on the surface of the base substrate metal containing a basic composition selected from a group consisting of titanium, zirconium and tantalum. This results in formation of a passive oxide film on the surface of the substrate material.

The optimum electrolytic conditions are the free sulfuric acid concentrations of 15-25 g./l. and the current density of 0.05-0.005 A./dm.<sup>2</sup>.

The anode of the invention satisfying the above optimum electrolytic conditions may be used in carrying out various kinds of electrolysis without being dissolved into electrolytes to soil them. Even when the anode of the invention is dissolved into the electrolyte, the solute is not deposited on the cathode so that it is possible to obtain an electrolytic product having a high purity.

The anode of the invention is low in the oxygen overvoltage during electrolysis so that the electrolysis can be carried out without consuming much electric power and, more particularly, can be applied to electrolytically obtain zinc containing little lead.

The invention will now be described with reference to examples.

A titanium plate having smooth surface whose thickness is 1 mm. and available in market and another titanium plate given sandblast treatment to form minute indentations on the surface thereof were used as substrates, respectively. These titanium plates with or without sandblast treatment were electrodeposited with manganese dioxide by means of electrolysis under the conditions shown in table 1 to obtain anodes. The characteristics of the anodes thus obtained were measured under the conditions shown in table 2. The results obtained are shown in table 3.

TABLE 1

| Composition of electrolyte |                                | Conditions for electrodeposition |                          |                                     |         |
|----------------------------|--------------------------------|----------------------------------|--------------------------|-------------------------------------|---------|
| Manganese sulfate          | H <sub>2</sub> SO <sub>4</sub> | Temperature                      | Current density          | Thickness of electrodeposited layer | Cathode |
| 150 g./l.                  | 20 g./l.                       | 90° C.                           | 0.01 A./dm. <sup>2</sup> | 20 $\mu$                            | Pb      |

TABLE 2

| Composition of electrolyte for zinc, g./l. |                                | Current density, A./dm. <sup>2</sup> |          | Temperature of electrolyte, °C. |              |
|--------------------------------------------|--------------------------------|--------------------------------------|----------|---------------------------------|--------------|
| Zn                                         | H <sub>2</sub> SO <sub>4</sub> | Mn <sup>++</sup>                     | At anode | At cathode                      | Cathode      |
| 50-75                                      | 150-190                        | 1                                    | 8.5      | 5.5                             | 36 Al plate. |

TABLE 3

| Anode                                                                                  | Time used, hrs. | Cell voltage, v. |
|----------------------------------------------------------------------------------------|-----------------|------------------|
| Titanium plate having smooth surface and electrodeposition with manganese dioxide.     | 16              | 4.2              |
| Titanium plate having minute indentations and electrodeposited with manganese dioxide. | 509             | 3.2              |

As seen from the Table 3, the anode made of the titanium plate having the smooth surface and electrodeposited with manganese dioxide was less durable and requires higher cell voltage than the anode made of the same titanium plate having minute indentations on the surface and electrodeposited with manganese dioxide; so that the former anode is not suitable

for practical use. The latter anode could be used as an insoluble anode for a considerably longer time, according to the conditions of electrodeposition.

But, the latter electrode produced gradually a film having a high electric resistance at the interface between the titanium substrate and the manganese dioxide layer to gradually increase the cell voltage.

The above-mentioned titanium plate whose surface was treated by sandblast to form minute indentations and the same titanium plate electroplated with a platinum layer having a thickness of 0.05  $\mu$  were electrodeposited with manganese dioxide under the electrodeposition conditions shown in the table 1 and the characteristics of the anodes thus obtained were measured under the conditions shown in the table 2.

15 The result obtained were shown in table 4.

TABLE 4

| Anode                                                                                                                                           | Time used, hrs. | Cell Voltage, v. |
|-------------------------------------------------------------------------------------------------------------------------------------------------|-----------------|------------------|
| Titanium plate having surface with minute indentations and electrodeposited with manganese dioxide.                                             | 500             | 3.2              |
| Titanium plate having surface with minute indentations and formed thereon with platinum layer and then electrodeposited with manganese dioxide. | >2,000          | 2.9              |

As seen from the above table 4, the titanium plate having the surface with minute indentations and formed thereon with the platinum layer and further electrodeposited with manganese dioxide required lower cell voltage and were more durable than the titanium plate having minute indentations on the surface and directly electrodeposited thereon with manganese dioxide.

35 The relation between the concentration of free sulfuric acid in the electrolyte used in the electrodeposition of manganese dioxide and the anode characteristics is shown in table 5 and the relation between the current density and the anode characteristics in table 6. The samples were titanium plates with minute indentations on the surface electroplated thereon with a platinum layer, of 0.05  $\mu$ -thick, and electrodeposited with manganese dioxide. The anode characteristics were measured under the conditions shown in the table 2.

45

TABLE 5

| Manganese sulfate | Free sulfuric acid | Current density electrodeposition, A./dm. <sup>2</sup> | Anode characteristics |                          |
|-------------------|--------------------|--------------------------------------------------------|-----------------------|--------------------------|
|                   |                    |                                                        | Cell voltage, v.      | Voltage increase, v./day |
| 150               | 5                  | 0.01                                                   | 3.0                   | 0.03                     |
| 150               | 10                 | 0.01                                                   | 2.9                   | 0.00                     |
| 150               | 20                 | 0.01                                                   | 2.9                   | 0.00                     |
| 150               | 30                 | 0.01                                                   | 2.9                   | 0.00                     |
| 150               | 50                 | 0.01                                                   | 3.1                   | 0.05                     |

TABLE 6

| Manganese sulfate | Free sulfuric acid | Current density electrodeposition, A./dm. <sup>2</sup> | Anode characteristics |                          |
|-------------------|--------------------|--------------------------------------------------------|-----------------------|--------------------------|
|                   |                    |                                                        | Cell voltage, v.      | Voltage increase, v./day |
| 150               | 20                 | 0.01                                                   | 2.9                   | 0.00                     |
| 150               | 20                 | 0.02                                                   | 2.9                   | 0.00                     |
| 150               | 20                 | 0.05                                                   | 3.3                   | 0.02                     |
| 150               | 20                 | 0.1                                                    | 3.6                   | 1.20                     |

70 As seen from the tables 5 and 6, it is necessary to use 10-30 g./l. of the concentration of the free sulfuric acid in the electrolyte for use in the electrodeposition of manganese dioxide and less than 0.05 A./dm.<sup>2</sup> of the current density for the purpose of obtaining the anode having excellent characteristics.

A titanium plate, a zirconium plate, a tantalum plate and Ti-1% Pd alloy plate, all having a thickness of 1 mm. and available in market, were used and were treated by sandblast

on the surface. The plates thus treated were immersed in concentrated hydrochloric acid and then the surfaces thereof were made clean. Subsequently, these plates were covered with a layer of platinum, palladium or rhodium, each having a thickness shown in table 7. The layer thus formed was electrodeposited with manganese dioxide under the conditions shown in table 8 to manufacture the anodes of the invention.

TABLE 7

| Covering process   | Thickness of layer ( $\mu$ ) |      |     |
|--------------------|------------------------------|------|-----|
|                    | Pt                           | Pd   | Rh  |
| Heat decomposition | 0.02                         | 0.03 | —   |
| Electrodeposition  | 0.03                         | 0.05 | 0.1 |

mainly been used as an anode for electrolytic winning of zinc, with the result that the electrolytic zinc obtained contained comparatively large amount of lead as impurities. Thus, it was rather difficult to obtain zinc containing less than 0.003 percent of lead and adapted to be used for die casting.

On the contrary, the anode of the invention was used to win electrolytic zinc containing extremely small amounts of lead or substantially containing no lead, with the result that this electrolytic zinc obtained was suitable as die casting material.

The anode of the invention was used at the anodic potential of about 1.52 v. vs. S.C.E. (Standard Carmel Electrode) so that the cell voltage becomes less than about 2.9 v. On the contrary, the conventional lead alloy electrode was used at the anode potential of about 1.70 v. vs. S.C.E. so that the cell volt-

TABLE 8

| Number | Composition of electrolyte (g./l.)                                                     | Cathode | Spacing between electrodes (cm.) | Conditions for electrolysis                                                                                                                 |
|--------|----------------------------------------------------------------------------------------|---------|----------------------------------|---------------------------------------------------------------------------------------------------------------------------------------------|
| 1.     | {MnSO <sub>4</sub> ·4H <sub>2</sub> O, 150.}<br>{H <sub>2</sub> SO <sub>4</sub> , 10.} | Pb      | 3                                | {Current density, 0.007 A./dm. <sup>2</sup> .}<br>{Temperature of electrolyte, 90° C.}<br>{Thickness of electrodeposited layer, 10 $\mu$ .} |
| 2.     | {MnSO <sub>4</sub> ·4H <sub>2</sub> O, 150.}<br>{H <sub>2</sub> SO <sub>4</sub> , 20.} | PB      | 3                                | {Current density, 0.01 A./dm. <sup>2</sup> .}<br>{Temperature of electrolyte, 90° C.}<br>{Thickness of electrodeposited layer, 20 $\mu$ .}  |
| 3.     | {MnSO <sub>4</sub> ·4H <sub>2</sub> O, 150.}<br>{H <sub>2</sub> SO <sub>4</sub> , 30.} | Pb      | 3                                | {Current density, 0.015 A./dm. <sup>2</sup> .}<br>{Temperature of electrolyte, 90° C.}<br>{Thickness of electrodeposited layer, 50 $\mu$ .} |

The anode thus obtained each showed a uniform electrodeposition of manganese dioxide which was dense and had an excellent adhesive property and thus the manganese dioxide layer was not detached from the substrate material even by roughly handling.

The anodes manufactured as above described, when each used for electrolysis carried out with a cathode of a titanium plate in aqueous solution containing 3 percent salt water and 20 percent sulfuric acid at 40° C. and the current density of 5 A./dm.<sup>2</sup>, withstood a long time of use without any defect.

A titanium plate was used and the surface thereof was treated by sandblast to form minute indentations thereon which were cleaned. The plate thus treated was electrodeposited with a platinum layer having a thickness of 0.05  $\mu$  under the conditions shown in table 9 and then further electrodeposited with a manganese dioxide layer under the conditions shown in No. 2 of the table 8. The anode thus obtained was used under the conditions shown in table 10 to obtain electrolytic zinc.

TABLE 9

| Composition of electrolyte (g./l.)                                                                                                                                                            | Anode | Condition for electrolysis                                                         |
|-----------------------------------------------------------------------------------------------------------------------------------------------------------------------------------------------|-------|------------------------------------------------------------------------------------|
| Pt(NH <sub>3</sub> ) <sub>2</sub> ·(NO <sub>2</sub> ) <sub>2</sub> , 16.5.<br>NH <sub>4</sub> NO <sub>3</sub> , 100.<br>H <sub>2</sub> SO <sub>4</sub> , 10.<br>NH <sub>4</sub> OH (28%), 50. | Pt    | {Temperature of electrolyte, 80° C.}<br>{Current density, 2 A./dm. <sup>2</sup> .} |

TABLE 10

| Composition of electrolyte                            | G./l. | Conditions for electrolysis                                                                                 |
|-------------------------------------------------------|-------|-------------------------------------------------------------------------------------------------------------|
| Beginning of electrolysis:<br>Zn ion (as sulfate).... | 75    | Cathode..... <sup>(1)</sup><br>Current density, A./dm. <sup>2</sup> :<br>Anode..... 8.5<br>Cathode..... 5.5 |
| H <sub>2</sub> SO <sub>4</sub> .....                  | 150   |                                                                                                             |
| Mn ion.....                                           | 1     |                                                                                                             |
| End of Electrolysis:<br>Zn ion.....                   | 50    | Temperature of Electrolyte, 36° C.                                                                          |
| H <sub>2</sub> SO <sub>4</sub> .....                  | 190   | Duration of electrolysis, hours 24                                                                          |
| Mn ion.....                                           | 1     | Spacing between electrodes, cm. 3                                                                           |

<sup>1</sup> Highly pure aluminum.

The zinc obtained was highly pure zinc containing less than 0.001 percent of lead. Heretofore, Pb-1% Ag alloy has

age becomes about 3.2 v. This shows that the invention can not only economize the electric power consumption but also ensure reduction of the rate of oxidation of manganese ion in the electrolyte at the anode owing to the fact that the anodic potential is low, thereby reducing the amount of manganese oxide crust to be produced. Moreover, the anode of the invention can be used as an anode for use in zinc electrolysis for a long time in a stabilized state since manganese ion present in the electrolyte serves to prevent wear of the manganese dioxide layer.

It will be understood that the invention is not limited to the examples described and that many modifications may be introduced therein without departing from the scope of the invention.

We Claim:

1. A method of manufacturing an insoluble anode for use in electrolytic winning of zinc, which comprises treating by sandblast a base substrate metal of titanium or its alloy to form minute indentations on the surface, electroplating on said base substrate metal a thin layer of platinum, and electrodepositing a layer of manganese dioxide on said thin layer in aqueous solution of manganese sulfate containing 10-30 g./l. of free sulfuric acid at a current density of 0.015-0.007 A./dm.<sup>2</sup>.
2. A method of manufacturing an insoluble anode for use in electrolytic winning of zinc in accordance with claim 1 wherein the concentration of free sulfuric acid in said aqueous solution of manganese sulfate is 15-25 g./l. and said current density is 0.05-0.005 A./dm.<sup>2</sup>.
3. An insoluble anode suitable for use in electrolysis which comprises three components

- a. a base substrate treated by sandblasting, said substrate being selected from the group consisting of titanium, zirconium and tantalum or alloys thereof;
- b. a thin metal layer formed on said substrate, said thin metal layer being selected from the group consisting of platinum, palladium and rhodium or alloys thereof; and
- c. an outermost layer of manganese dioxide electroplated on said thin metal layer in an aqueous solution of manganese sulfate containing about 10 to about 30 g./l. of free sulfuric acid at a current density of about 0.015 to about 0.007 A./dm.<sup>2</sup>.

4. The insoluble anode of claim 3 wherein the thickness of said thin metal layer (b) is 0.01 to 0.3  $\mu$  and the thickness of said manganese dioxide layer (c) is 10 to 100  $\mu$ .